



US010551761B2

(12) **United States Patent**  
**Kubo et al.**

(10) **Patent No.:** **US 10,551,761 B2**  
(45) **Date of Patent:** **\*Feb. 4, 2020**

(54) **TONER FOR ELECTROPHOTOGRAPHY**

(71) Applicant: **KAO CORPORATION**, Tokyo (JP)

(72) Inventors: **Takashi Kubo**, Wakayama (JP); **Kota Ijichi**, Wakayama (JP)

(73) Assignee: **KAO CORPORATION**, Tokyo (JP)

(\*) Notice: Subject to any disclaimer, the term of this patent is extended or adjusted under 35 U.S.C. 154(b) by 0 days.

This patent is subject to a terminal disclaimer.

(21) Appl. No.: **16/077,241**

(22) PCT Filed: **Feb. 9, 2017**

(86) PCT No.: **PCT/JP2017/004769**

§ 371 (c)(1),

(2) Date: **Aug. 10, 2018**

(87) PCT Pub. No.: **WO2017/141816**

PCT Pub. Date: **Aug. 24, 2017**

(65) **Prior Publication Data**

US 2019/0064687 A1 Feb. 28, 2019

(30) **Foreign Application Priority Data**

Feb. 16, 2016 (JP) ..... 2016-027237  
Feb. 9, 2017 (JP) ..... 2017-021856

(51) **Int. Cl.**

**G03G 9/08** (2006.01)  
**G03G 9/097** (2006.01)  
**G03G 9/087** (2006.01)

(52) **U.S. Cl.**

CPC ..... **G03G 9/09775** (2013.01); **G03G 9/081** (2013.01); **G03G 9/08755** (2013.01)

(58) **Field of Classification Search**

CPC ..... G03G 9/09755  
USPC ..... 430/108.2

See application file for complete search history.

(56) **References Cited**

U.S. PATENT DOCUMENTS

2011/0097664 A1 4/2011 Nosella et al.  
2013/0244173 A1 9/2013 Qiu et al.

FOREIGN PATENT DOCUMENTS

|    |               |         |
|----|---------------|---------|
| JP | 4-273255 A    | 9/1992  |
| JP | 5-241374 A    | 9/1993  |
| JP | 2000-318391 A | 11/2000 |
| JP | 2000-336163 A | 12/2000 |
| JP | 2009-157017 A | 7/2009  |
| JP | 2012-126898 A | 7/2012  |
| JP | 2015-121579 A | 7/2015  |

OTHER PUBLICATIONS

International Search Report dated Apr. 25, 2017 in PCT/JP2017/004769 filed Feb. 9, 2017.

Extended European Search Report dated Aug. 2, 2019, in Patent Application No. 17753074.8, citing documents AO-AP therein, 7 pages.

*Primary Examiner* — Mark A Chapman

(74) *Attorney, Agent, or Firm* — Oblon, McClelland, Maier & Neustadt, L.L.P.

(57) **ABSTRACT**

To provide a toner for electrophotography exhibiting an excellent charge rise property, and a process for producing the same.

[1] A toner for electrophotography containing a binder resin, and a polyhydroxyamine compound represented by the following formula (1) in an amount of 0.001 part by mass or more and 5.0 parts by mass or less per 100 parts by mass of the binder resin, and [2] a process for producing a toner for electrophotography, including: melt-kneading a toner raw material mixture containing a binder resin, and a polyhydroxyamine compound represented by the following formula (1) in an amount of 0.001 part by mass or more and 5.0 parts by mass or less per 100 parts by mass of the binder resin; and pulverizing a resulting melt-kneaded material.

**16 Claims, No Drawings**

## 1

## TONER FOR ELECTROPHOTOGRAPHY

## FIELD OF THE INVENTION

The present invention relates to a toner for electrophotography and a process for producing the same.

## BACKGROUND OF THE INVENTION

According to the speeding up and energy saving of printers and duplicators in recent years, a toner capable of responding to the demand is becoming increasingly necessary.

PTL 1 describes about a production process of a binder component of a toner for electrophotography. The literature targets to achieve such demands that, for example, fusing is performed at a lower temperature, offset is prevented at a higher temperature, a stable image is formed even though the environmental conditions, such as the humidity, largely fluctuate, and excellent charge rise is achieved. PTL 1 describes a production process of a carbodiimide-modified polyester resin characterized by reacting a polyester resin (A) and a carbodiimide group-containing compound (B).

PTL 1: JP 2000-336163 A

## SUMMARY OF THE INVENTION

The present invention relates to the following items [1] and [2].

[1] A toner for electrophotography, containing a binder resin, and a polyhydroxyamine compound represented by the following formula (1) in an amount of 0.001 part by mass or more and 5.0 parts by mass or less per 100 parts by mass of the binder resin:



wherein  $\text{R}^1$  represents a hydrogen atom, an alkyl group having a number of carbon atoms of 1 or more and 5 or less, or a hydroxyalkyl group having a number of carbon atoms of 1 or more and 5 or less;  $\text{R}^2$  represents a hydrogen atom, an alkyl group having a number of carbon atoms of 1 or more and 6 or less, or a hydroxyalkyl group having a number of carbon atoms of 1 or more and 5 or less; and  $\text{R}^3$  and  $\text{R}^4$  each represent an alkanediyl group having a number of carbon atoms of 1 or more and 5 or less, provided that  $\text{R}^3$  and  $\text{R}^4$  may be the same as or different from each other.

[2] A process for producing a toner for electrophotography, including: melt-kneading a toner raw material mixture containing a binder resin, and a polyhydroxyamine compound represented by the formula (1) in an amount of 0.001 part by mass or more and 5.0 parts by mass or less per 100 parts by mass of the binder resin; and pulverizing a resulting melt-kneaded material.

## DETAILED DESCRIPTION OF THE INVENTION

When high-speed printing is performed, it is necessary that the toner is rapidly charged, i.e., is excellent in charge rise property. However, there is a demand of further

## 2

improvement of the toner for electrophotography described in PTL 1 from the standpoint of the charge rise property.

The present invention relates to a toner for electrophotography exhibiting an excellent charge rise property, and a process for producing the same.

It has been found that the charge rise property of the toner for electrophotography is increased by adding a particular polyhydroxyamine compound to the toner.

The present invention relates to the following items [1] and [2].

[1] A toner for electrophotography containing a binder resin, and a polyhydroxyamine compound represented by the following formula (1) in an amount of 0.001 part by mass or more and 5.0 parts by mass or less per 100 parts by mass of the binder resin:



wherein  $\text{R}^1$  represents a hydrogen atom, an alkyl group having a number of carbon atoms of 1 or more and 5 or less, or a hydroxyalkyl group having a number of carbon atoms of 1 or more and 5 or less;  $\text{R}^2$  represents a hydrogen atom, an alkyl group having a number of carbon atoms of 1 or more and 6 or less, or a hydroxyalkyl group having a number of carbon atoms of 1 or more and 5 or less; and  $\text{R}^3$  and  $\text{R}^4$  each represent an alkanediyl group having a number of carbon atoms of 1 or more and 5 or less, provided that  $\text{R}^3$  and  $\text{R}^4$  may be the same as or different from each other.

[2] A process for producing a toner for electrophotography, including: melt-kneading a toner raw material mixture containing a binder resin, and a polyhydroxyamine compound represented by the formula (1) in an amount of 0.001 part by mass or more and 5.0 parts by mass or less per 100 parts by mass of the binder resin; and pulverizing a resulting melt-kneaded material.

According to the present invention, a toner for electrophotography exhibiting an excellent charge rise property, and a process for producing the same can be provided. According to the present invention, furthermore, a toner for electrophotography having an excellent odor suppression capability against odors derived from the binder resin and the like, and a process for producing the same can be provided.

## [Toner for Electrophotography]

The toner for electrophotography of the present invention contains a binder resin, and a polyhydroxyamine compound represented by the following formula (1) (which may be hereinafter referred simply to as a "polyhydroxyamine compound") in an amount of 0.001 part by mass or more and 5.0 parts by mass or less per 100 parts by mass of the binder resin:



wherein  $\text{R}^1$  represents a hydrogen atom, an alkyl group having a number of carbon atoms of 1 or more and 5 or less,

or a hydroxyalkyl group having a number of carbon atoms of 1 or more and 5 or less; R<sup>2</sup> represents a hydrogen atom, an alkyl group having a number of carbon atoms of 1 or more and 6 or less, or a hydroxyalkyl group having a number of carbon atoms of 1 or more and 5 or less; and R<sup>3</sup> and R<sup>4</sup> each represent an alkanediyl group having a number of carbon atoms of 1 or more and 5 or less, provided that R<sup>3</sup> and R<sup>4</sup> may be the same as or different from each other.

According to the present invention, a toner for electrophotography exhibiting an excellent charge rise property can be obtained.

While the reason therefor is not clear, it can be estimated that the polyhydroxyamine compound contains in the molecule thereof an amino group having a tendency to hold a positive charge and a hydroxy group having a tendency to hold a negative charge, and therefore the toner can be rapidly charged through the charge shift from the amino group to the hydroxy group for the negatively charged toner, or the charge shift from the hydroxy group to the amino group for the positively charged toner.

<Polyhydroxyamine Compound>

The polyhydroxyamine compound is a compound represented by the following formula (1) from the standpoint of the excellent charge rise property and the excellent odor suppression capability.



wherein R<sup>1</sup> represents a hydrogen atom, an alkyl group having a number of carbon atoms of 1 or more and 5 or less, or a hydroxyalkyl group having a number of carbon atoms of 1 or more and 5 or less; R<sup>2</sup> represents a hydrogen atom, an alkyl group having a number of carbon atoms of 1 or more and 6 or less, or a hydroxyalkyl group having a number of carbon atoms of 1 or more and 5 or less; and R<sup>3</sup> and R<sup>4</sup> each represent an alkanediyl group having a number of carbon atoms of 1 or more and 5 or less, provided that R<sup>3</sup> and R<sup>4</sup> may be the same as or different from each other.

The number of carbon atoms of the alkyl group of R<sup>1</sup> is preferably 4 or less, more preferably 3 or less, further preferably 2 or less, and still further preferably 1, from the standpoint of providing the excellent charge rise property.

The alkyl group of R<sup>1</sup> may be any of straight-chain and branched-chain, examples of which include a methyl group, an ethyl group, a n-propyl group, an isopropyl group, various butyl groups, and various pentyl groups, and is preferably at least one selected from a methyl group and an ethyl group, and more preferably a methyl group.

The number of carbon atoms of the hydroxyalkyl group of R<sup>1</sup> is preferably 4 or less, more preferably 3 or less, further preferably 2 or less, and still further preferably 1, from the standpoint of providing the excellent charge rise property.

Examples of the hydroxyalkyl group of R<sup>1</sup> include a hydroxymethyl group, a 2-hydroxyethyl group, a 2-hydroxypropyl group, a 3-hydroxypropyl group, a 2-hydroxybutyl group, a 3-hydroxybutyl group, and a 4-hydroxybutyl group, and the hydroxyalkyl group is preferably at least one selected from a hydroxymethyl group and a 2-hydroxyethyl group, and more preferably a hydroxymethyl group.

Among these, R<sup>1</sup> is preferably an alkyl group having a number of carbon atoms of 1 or more and 3 or less or a

hydroxyalkyl group having a number of carbon atoms of 1 or more and 3 or less, more preferably at least one selected from a methyl group, an ethyl group, a hydroxymethyl group, and a hydroxyethyl group, and further preferably a hydroxymethyl group.

The number of carbon atoms of the alkyl group of R<sup>2</sup> is preferably 3 or less, and more preferably 2 or less, and is preferably 1 or more.

The alkyl group of R<sup>2</sup> may be any of straight-chain, branched-chain, and cyclic, examples of which include a methyl group, an ethyl group, a n-propyl group, an isopropyl group, every kind of butyl groups, every kind of pentyl groups, every kind of hexyl groups, a cyclopentyl group, and a cyclohexyl group.

The number of carbon atoms of the hydroxyalkyl group of R<sup>2</sup> is preferably 3 or less, and more preferably 2 or less, and is preferably 1 or more. Examples of the hydroxyalkyl group of R<sup>2</sup> include the same compounds described above for R<sup>1</sup>.

Among these, R<sup>2</sup> is preferably a hydrogen atom, an alkyl group having a number of carbon atoms of 1 or more and 3 or less, or a hydroxyalkyl group having a number of carbon atoms of 1 or more and 3 or less, more preferably a hydrogen atom.

The number of carbon atoms of the alkanediyl group of R<sup>3</sup> and R<sup>4</sup> is preferably 4 or less, more preferably 3 or less, further preferably 2 or less, and still further preferably 1.

Examples of the alkanediyl group of R<sup>3</sup> and R<sup>4</sup> include a methylene group, an ethylene group, a trimethylene group, a propan-1,2-diy group, and a tetramethylene group, and a methylene group is preferred.

Specific examples of the polyhydroxyamine compound include 2-amino-1,3-propanediol, 2-amino-2-methyl-1,3-propanediol, 2-amino-2-ethyl-1,3-propanediol, 2-amino-2-hydroxymethyl-1,3-propanediol, 2-amino-2-hydroxyethyl-1,3-propanediol, 4-amino-4-hydroxypropyl-1,7-heptanediol, 2-(N-ethyl)amino-1,3-propanediol, 2-(N-ethyl)amino-2-hydroxymethyl-1,3-propanediol, 2-(N-decyl)amino-1,3-propanediol, and 2-(N-decyl)amino-2-hydroxymethyl-1,3-propanediol.

Among these, the polyhydroxyamine compound is preferably at least one selected from 2-amino-2-hydroxymethyl-1,3-propanediol, 2-amino-2-hydroxyethyl-1,3-propanediol, 2-amino-1,3-propanediol, 2-amino-2-methyl-1,3-propanediol, and 2-amino-2-ethyl-1,3-propanediol, more preferably at least one selected from 2-amino-2-hydroxymethyl-1,3-propanediol, 2-amino-2-hydroxyethyl-1,3-propanediol, and 2-amino-2-methyl-1,3-propanediol, and further preferably 2-amino-2-hydroxymethyl-1,3-propanediol, from the standpoint of providing the excellent charge rise property.

One kind or two or more kinds of the polyhydroxyamine compound may be used. The polyhydroxyamine compound can be produced by an ordinary method.

The content of the polyhydroxyamine compound is 0.001 part by mass or more and 5.0 parts by mass or less from the standpoint of providing the excellent charge rise property, is preferably 0.01 part by mass or more, more preferably 0.03 part by mass or more, further preferably 0.1 part by mass or more, and still further preferably 0.3 part by mass or more, and is preferably 4.0 parts by mass or less, and more preferably 3.0 parts by mass or less, from the standpoint of providing the excellent charge rise property, all per 100 parts by mass of the total amount of the binder resin of the toner for electrophotography.

<Binder Resin>

Examples of the binder resin include a polycondensation resin, such as a polyester and a polyamide, a styrene resin, such as a styrene resin and a styrene-acrylic resin, an epoxy

resin, a polycarbonate, a polyurethane, and a composite resin of these resins. Examples of the composite resin include a polyester-polyamide, and a composite resin having a polyester segment. Examples of the composite resin having a polyester segment include a composite resin having a polyester segment and a styrene resin segment, and a urethane-modified polyester resin.

In the present invention, the binder resin is preferably a resin having a polyester moiety obtained through polycondensation of an alcohol component and a carboxylic acid component, or a styrene resin, more preferably at least one selected from a urethane-modified polyester resin, a polyester, a styrene resin, and a composite resin having a polyester segment and a styrene resin segment, further preferably at least one selected from a polyester, a styrene resin, and a composite resin having a polyester segment and a styrene resin segment, and still further preferably at least one selected from a polyester and a composite resin having a polyester segment and a styrene resin segment, from the standpoint of the durability and the low-temperature fusing property.

The binder resin is preferably at least one selected from a polyester and a composite resin having a polyester segment from the standpoint of enhancing the charge rise property. [Polyester]

The polyester is preferably obtained through polycondensation of a raw material monomer containing an alcohol component containing a dihydric or higher hydric alcohol and a carboxylic acid component containing dibasic or higher basic carboxylic acid.

The alcohol component may be any of an aromatic polyol compound and an aliphatic polyol compound.

The aromatic polyol compound is preferably an alkylene oxide adduct of bisphenol A, and more preferably an alkylene oxide adduct of bisphenol A represented by the formula (I):

(I)



wherein RO and OR each represent an oxyalkylene group, R represents at least one selected from an ethylene group and a propylene group, and x and y each represent an average addition molar number of alkylene oxide, and each are a positive number, provided that the sum of x and y is 1 or more, and preferably 1.5 or more, and is 16 or less, preferably 8 or less, and more preferably 4 or less, from the standpoint of the durability and the charge rise property.

Examples of the alkylene oxide adduct of bisphenol A represented by the formula (I) include a propylene oxide adduct of 2,2-bis(4-hydroxyphenyl)propane and an ethylene oxide adduct of 2,2-bis(4-hydroxyphenyl)propane. One kind or two or more kinds of the compound may be used.

The content of the alkylene oxide adduct of bisphenol A represented by the formula (I) is preferably 70% by mol or more, more preferably 90% by mol or more, further preferably 95% by mol or more, and still further preferably 100% by mol, based on the alcohol component.

Examples of the aliphatic polyol compound is preferably an aliphatic diol having a number of carbon atoms of 2 or

more and 20 or less and a trihydric or higher hydric aliphatic alcohol, such as glycerin, and among these, an aliphatic diol is preferred.

Examples of the aliphatic diol include ethylene glycol, 1,2-propanediol, 1,3-propanediol, 1,4-butanediol, 1,5-pentanediol, 1,6-hexanediol, 1,4-butenediol, 1,3-butanediol, neopentyl glycol, 1,10-decanediol, and 1,12-dodecanediol.

The content of the aliphatic diol is preferably 70% by mol or more, more preferably 90% by mol or more, further preferably 95% by mol or more, and still further preferably 100% by mol, based on the alcohol component.

As for the carboxylic acid component, the dibasic carboxylic acid is preferably an aromatic dicarboxylic acid from the standpoint of the storage stability, and is preferably an aliphatic dicarboxylic acid from the standpoint of the low-temperature fusing property.

Examples of the aromatic dicarboxylic acid include phthalic acid, isophthalic acid, terephthalic acid, and an anhydride of these acids or an alkyl (having from 1 to 3 carbon atoms) ester of these acids, and among these, terephthalic acid and isophthalic acid are more preferred, and terephthalic acid is further preferred. One kind or two or more kinds thereof may be used. In the present invention, the carboxylic acid component includes not only a free acid but also an anhydride forming an acid through decomposition during reaction and an ester with an alkyl having from 1 to 3 carbon atoms.

The content of the aromatic dicarboxylic acid is preferably 10% by mol or more, more preferably 30% by mol or more, and further preferably 50% by mol or more, and may be 100% by mol or less, based on the carboxylic acid component.

Examples of the aliphatic dicarboxylic acid include an aliphatic dicarboxylic acid, such as oxalic acid, malonic acid, maleic acid, fumaric acid, citraconic acid, itaconic acid, glutaconic acid, succinic acid, adipic acid, and succinic acid substituted with an alkyl group having from 1 to 20 carbon atoms or an alkenyl group having from 2 to 20 carbon atoms, such as dodecenylsuccinic acid and octylsuccinic acid; and anhydrides of these acids and alkyl (having from 1 to 3 carbon atoms) esters of these acids. One kind or two or more kinds thereof may be used.

The content of the aliphatic dicarboxylic acid is preferably 10% by mol or more, and more preferably 20% by mol or more, and, from the standpoint of the charge rise property, is preferably 90% by mol or less, and more preferably 80% by mol or less, based on the carboxylic acid component.

The carboxylic acid component preferably contains a tribasic or higher basic carboxylic acid from the standpoint of the productivity.

Examples of the tribasic or higher basic carboxylic acid include 1,2,4-benzenetricarboxylic acid (trimellitic acid), 2,5,7-naphthalenetricarboxylic acid, pyromellitic acid, and anhydrides of these acids and lower alkyl (having from 1 to 3 carbon atoms) esters of these acids, and among these, trimellitic acid and an anhydride thereof are preferred.

The content of the tribasic or higher basic carboxylic acid, preferably the content of trimellitic acid or trimellitic anhydride, is preferably 5% by mol or more, more preferably 10% by mol or more, and further preferably 15% by mol or more, and is preferably 50% by mol or less, more preferably 40% by mol or less, further preferably 35% by mol or less, and still further preferably 30% by mol or less, from the standpoint of the low-temperature fusing property, based on the carboxylic acid component.

A monohydric alcohol may be contained in the alcohol component, and a monobasic carboxylic acid may be con-

tained in the carboxylic acid component, appropriately from the standpoint of the control of the molecular weight.

The equivalent ratio (COOH group/OH group) of the carboxylic acid component and the alcohol component is preferably 0.7 or more, and more preferably 0.8 or more, and is preferably 1.3 or less, and more preferably 1.2 or less, from the standpoint of controlling the end group.

The polycondensation of the alcohol component and the carboxylic acid component may be performed, for example, in an inert gas atmosphere, in the presence of an esterification catalyst, a polymerization inhibitor, or the like depending on necessity, at a temperature of approximately 180° C. or more and 250° C. or less. Examples of the esterification catalyst include a tin compound, such as dibutyltin oxide and tin(II) 2-ethylhexanoate, and a titanium compound, such as titanium diisopropylate bistrithanolamine. Examples of an esterification promoter used with the esterification catalyst include gallic acid. The amount of the esterification catalyst used is preferably 0.01 part by mass or more, and more preferably 0.1 part by mass or more, and is preferably 1 parts by mass or less, and more preferably 0.6 part by mass or less, per 100 parts by mass of the total amount of the alcohol component and the carboxylic acid component. The amount of the esterification promoter used is preferably 0.001 part by mass or more, and more preferably 0.01 part by mass or more, and is preferably 0.5 part by mass or less, and more preferably 0.1 part by mass or less, per 100 parts by mass of the total amount of the alcohol component and the carboxylic acid component.

[Styrene Resin]

The styrene resin is preferably obtained through addition polymerization of a raw material monomer containing a styrene compound.

The styrene compound used may be styrene and a styrene derivative, such as  $\alpha$ -methylstyrene and vinyltoluene (and in the following description, styrene and a styrene derivative are collectively referred to as a "styrene compound").

The content of the styrene compound is preferably 50% by mass or more, more preferably 60% by mass or more, further preferably 70% by mass or more, and still further preferably 75% by mass or more, from the standpoint of the durability, and is preferably 95% by mass or less, more preferably 90% by mass or less, and further preferably 87% by mass or less, from the standpoint of the low-temperature fusing property, based on the raw material monomer of the styrene resin.

Examples of the raw material monomer of the styrene resin other than the styrene compound include an alkyl (meth)acrylate ester; an ethylenic unsaturated monoolefin compound, such as ethylene and propylene; a diolefin compound, such as butadiene; a halogenated vinyl compound, such as vinyl chloride; a vinyl ester compound, such as vinyl acetate and vinyl propionate; an ethylenic monocarboxylate ester, such as dimethylaminoethyl (meth)acrylate; a vinyl ether compound, such as vinyl methyl ether; a vinylidene halide compound, such as vinylidene chloride; and an N-vinyl compound, such as N-vinylpyrrolidone.

Two or more kinds of the raw material monomer of the styrene resin other than the styrene compound may be used. In the description herein, the "(meth)acrylic acid" means at least one selected from acrylic acid and methacrylic acid.

The raw material monomer of the styrene resin other than the styrene compound is preferably an alkyl (meth)acrylate ester from the standpoint of enhancing the low-temperature fusing property of the toner. The number of carbon atoms of the alkyl group in the alkyl (meth)acrylate ester is preferably 1 or more, more preferably 2 or more, and further preferably

3 or more, and is preferably 22 or less, more preferably 18 or less, further preferably 12 or less, and still further preferably 8 or less, from the aforementioned standpoint. The number of carbon atoms of the alkyl ester means the number of carbon atoms derived from the alcohol component constituting the ester.

Specific examples of the alkyl (meth)acrylate ester include methyl (meth)acrylate, ethyl (meth)acrylate, (iso) propyl (meth)acrylate, 2-hydroxyethyl (meth)acrylate, (iso) or tert-butyl (meth)acrylate, 2-ethylhexyl (meth)acrylate, (iso)octyl (meth)acrylate, (iso)decyl (meth)acrylate, and (iso)stearyl (meth)acrylate. The expressions "(iso- or tert-)" and "(iso)" herein each mean that both the case where the prefix exists and the case where the prefix does not exist are included, and the case where the prefix does not exist shows the normal. The "(meth)acrylate" means that both the cases of an acrylate and a methacrylate are included.

The content of the alkyl (meth)acrylate ester is preferably 5% by mass or more, more preferably 10% by mass or more, and further preferably 13% by mass or more, from the standpoint of the low-temperature fusing property, and is preferably 50% by mass or less, more preferably 40% by mass or less, further preferably 30% by mass or less, and still further preferably 25% by mass or less, from the same standpoint, based on the raw material monomer of the styrene resin segment.

The resin obtained through addition polymerization of the raw material monomer containing the styrene compound and the alkyl (meth)acrylate ester may also be referred to as a styrene-(meth)acrylate resin.

The addition polymerization reaction of the raw material monomer of the styrene resin may be performed, for example, by an ordinary method in the presence of a polymerization initiator, such as dicumyl peroxide, a cross-linking agent, and the like, in the presence of an organic solvent or without a solvent, and the temperature condition is preferably 110° C. or more, more preferably 120° C. or more, and further preferably 130° C. or more, and is preferably 250° C. or less, more preferably 200° C. or less, and further preferably 170° C. or less.

In the case where an organic solvent is used in the addition polymerization reaction, xylene, toluene, methyl ethyl ketone, acetone, and the like may be used. The amount of the organic solvent used is preferably 10 parts by mass or more and 50 parts by mass or less per 100 parts by mass of the raw material monomer of the styrene resin.

[Composite Resin]

The composite resin preferably has a polyester segment and a styrene resin segment.

The polyester segment may be formed of a polyester, and preferred examples of the polyester include the same ones described above for the polyester.

The styrene resin segment may be formed of a styrene resin, and preferred examples of the styrene resin include the same ones described above for the styrene resin.

In the case where the raw material monomer of the styrene resin segment contains an alkyl (meth)acrylate ester, the number of carbon atoms of the alkyl group in the alkyl (meth)acrylate ester is preferably 6 or more, and more preferably 8 or more, and is preferably 22 or less, and more preferably 18 or less, from the aforementioned standpoint. The number of carbon atoms of the alkyl ester means the number of carbon atoms derived from the alcohol component constituting the ester.

The composite resin is preferably a composite resin that is obtained by further using a bireactive monomer capable of reacting with both the raw material monomer of the poly-

ester segment and the raw material monomer of the styrene resin segment, in addition to the raw material monomer of the polyester segment and the raw material monomer of the styrene resin segment, from the standpoint of enhancing the durability and the low-temperature fusing property of the toner. Accordingly, in the production of the composite resin through polymerization of the raw material monomer of the polyester segment and the raw material monomer of the styrene resin segment, the polycondensation reaction and/or the addition polymerization reaction are preferably performed in the presence of the bireactive monomer. According to the procedure, the composite resin becomes such a composite resin that the polyester segment and the styrene resin segment are bonded to each other through the constitutional unit derived from the bireactive monomer, and the polyester segment and the styrene resin segment are dispersed finely and uniformly.

Accordingly, the composite resin is preferably a resin obtained through polymerization of (i) the raw material monomer of the polyester segment containing an alcohol component containing the alkylene oxide adduct of bisphenol A represented by the formula (I), and a carboxylic acid component containing an aromatic dicarboxylic acid, (ii) the raw material monomer of the styrene resin segment, and (iii) the bireactive monomer capable of reacting with both the raw material monomer of the polyester segment and the raw material monomer of the styrene resin segment, from the standpoint of enhancing the durability and the low-temperature fusing property of the toner.

The bireactive monomer is preferably a compound that has in the molecule thereof at least one functional group selected from a hydroxy group, a carboxy group, an epoxy group, a primary amino group, and a secondary amino group, preferably at least one functional group selected from a hydroxy group and a carboxy group, and more preferably a carboxy group and an ethylenic unsaturated bond, and the use of the bireactive monomer may enhance the dispersibility of the resin as the dispersed state. The bireactive monomer is preferably at least one selected from acrylic acid, methacrylic acid, fumaric acid, maleic acid, and maleic anhydride, and is more preferably acrylic acid, methacrylic acid, or fumaric acid, and further preferably acrylic acid or methacrylic acid, from the standpoint of the reactivity of the polycondensation reaction and the addition polymerization reaction. In the use thereof with a polymerization inhibitor, a polybasic carboxylic acid having an ethylenic unsaturated bond, such as fumaric acid, functions as a raw material monomer of the polyester segment. In this case, fumaric acid or the like is not the bireactive monomer but is a raw material monomer of the polyester segment.

The amount of the bireactive monomer used is preferably 1 mole or more, more preferably 2 moles or more, and further preferably 3 moles or more, from the standpoint of the low-temperature fusing property, and is preferably 20 moles or less, more preferably 10 moles or less, and further preferably 7 moles or less, from the standpoint of the durability of the toner, per 100 moles in total of the alcohol component of the polyester segment.

The mass ratio (polyester segment/styrene resin segment) of the polyester segment and the styrene resin segment in the composite resin is preferably 60/40 or more, more preferably 70/30 or more, and further preferably 75/25 or more, from the standpoint of the low-temperature fusing property, and is preferably 95/5 or less, more preferably 90/10 or less, and further preferably 85/15 or less, from the standpoint of the durability. In the aforementioned calculation, the mass of the polyester segment is the amount obtained by subtracting the

amount (calculated amount) of water eliminated in the polycondensation reaction from the mass of the raw material monomer of the polycondensation resin used, and the amount of the bireactive monomer is included in the amount of the raw material monomer of the polyester segment. The amount of the styrene resin segment is the amount of the raw material monomer of the styrene resin segment, and the amount of the polymerization initiator is included in the amount of the raw material monomer of the styrene resin segment.

[Urethane-Modified Polyester Resin]

Examples of the urethane-modified polyester resin include a urethane-modified polyester resin obtained through reaction of one kind or two or more kinds of a polyester and a polyisocyanate compound, from the standpoint of enhancing the durability.

The valence of the polyisocyanate compound is preferably 2 or more, and is preferably 8 or less, more preferably 6 or less, and further preferably 4 or less.

Examples of the polyisocyanate compound include a diisocyanate compound, such as an aliphatic diisocyanate and an aromatic diisocyanate, and prepolymer type, an isocyanurate type, urea type, and carbodiimide type derivatives of the diisocyanate compound.

Examples of the aliphatic diisocyanate compound include isophorone diisocyanate, 4,4'-dicyclohexylmethane diisocyanate, 4-methyl-1,3-cyclohexylene diisocyanate, and 1,2-bis(isocyanatomethyl)cyclohexanehexamethylene diisocyanate.

Examples of the aromatic diisocyanate compound include 4,4'-diphenylmethane diisocyanate, 2,4-tolylene diisocyanate, 2,6-tolylene diisocyanate, m-phenylene diisocyanate, p-phenylene diisocyanate, 1,3-xylylene diisocyanate, 1,4-xylylene diisocyanate, 1,5-naphthalene diisocyanate, and 3,3'-dimethyl-4,4'-biphenylene diisocyanate.

The urethane-modified polyester resin may be obtained by an ordinary method, and can be obtained, for example, by adding and reacting a polyisocyanate compound to a melt mixture of one kind or two or more kinds of polyesters.

The amount of the polyisocyanate compound added is preferably 0.1 part by mass or more, more preferably 0.5 part by mass or more, and further preferably 1.0 part by mass or more, and is preferably 20 parts by mass or less, more preferably 15 parts by mass or less, and further preferably 10 parts by mass or less, per 100 parts by mass of the polyester resin.

<Properties of Binder Resin>

The softening point of the binder resin is preferably 90° C. or more, more preferably 95° C. or more, and further preferably 100° C. or more, from the standpoint of enhancing the durability and the hot offset resistance, and is preferably 150° C. or less, more preferably 145° C. or less, and further preferably 140° C. or less, from the standpoint of enhancing the low-temperature fusing property of the toner.

The glass transition temperature of the binder resin is preferably 45° C. or more, more preferably 50° C. or more, and further preferably 55° C. or more, from the standpoint of enhancing the durability and the storage stability, and is preferably 80° C. or less, more preferably 75° C. or less, further preferably 70° C. or less, and still further preferably 65° C. or less, from the standpoint of enhancing the low-temperature fusing property of the toner.

The acid value of the binder resin is preferably 40 mgKOH/g or less, more preferably 30 mgKOH/g or less, and further preferably 20 mgKOH/g or less, and is preferably 1 mgKOH/g or more, and more preferably 2 mgKOH/g

## 11

or more, from the standpoint of enhancing the environmental stability of the charge amount of the toner.

The number average molecular weight of the binder resin is preferably 1,000 or more, more preferably 1,500 or more, and further preferably 3,000 or more, and is preferably 7,000 or less, more preferably 6,000 or less, and further preferably 5,500 or less, from the standpoint of the durability and the storage stability.

The measurement methods of the softening point, the glass transition temperature, the acid value, and the number average molecular weight are the methods described in the examples. In the case where two or more kinds of resins are contained, the softening point, the glass transition temperature, the acid value, and the number average molecular weight are preferably such values that the weighted average values thereof are in the aforementioned ranges respectively. [Resins H and L]

In the aforementioned resins, the toner of the present invention preferably contains two kinds of resins having softening points that are different from each other by 20° C. or more from the standpoint of the high-temperature offset resistance and the low-temperature fusing property.

The softening point of the resin H having a higher softening point is preferably 170° C. or less, and more preferably 160° C. or less, from the standpoint of the low-temperature fusing property, and is preferably 110° C. or more, more preferably 120° C. or more, and further preferably 130° C. or more, from the standpoint of the high-temperature offset resistance.

The softening point of the resin L having a lower softening point is preferably 80° C. or more, and more preferably 95° C. or more, from the standpoint of the durability, and is preferably 125° C. or less, and more preferably 115° C. or less, from the standpoint of the low-temperature fusing property.

The difference in softening point between the resin H and the resin L is preferably 10° C. or more, more preferably 20° C. or more, further preferably 25° C. or more, and still further preferably 30° C. or more, and is preferably 60° C. or less, more preferably 50° C. or less, and further preferably 40° C. or less, from the standpoint of the high-temperature offset resistance and the low-temperature fusing property.

The mass ratio (resin H/resin L) of the resin H and the resin L is preferably 20/80 or more, more preferably 40/60 or more, further preferably 50/50 or more, and still further preferably 60/40 or more, from the standpoint of the durability and the productivity, and is preferably 90/10 or less, more preferably 80/20 or less, and further preferably 75/25 or less, from the standpoint of the low-temperature fusing property.

The resin H and the resin L each are preferably an amorphous resin.

In the present invention, the "amorphous resin" means a resin that has a value of a crystallinity index, which is defined by the ratio of the softening point (° C.) with respect to the highest endothermic peak temperature (° C.) with a differential scanning calorimeter (DSC), i.e.,  $((\text{softening point}) / (\text{highest endothermic peak temperature}))$ , of 1.4 or more or less than 0.6. The highest endothermic peak temperature means the temperature of the peak that has the highest temperature among the endothermic peaks observed under the condition of the measurement method described in the examples.

In the case where the resin H and the resin L each are an amorphous resin, the amorphous resin is preferably a resin containing an aromatic polyol as the alcohol component among the aforementioned resins. The preferred examples

## 12

of the aromatic polyol compound and the other preferred examples are the same as the examples described above. [Resin C]

In the aforementioned resins, the toner of the present invention preferably contains a crystalline resin C (which may be hereinafter referred simply to as a "resin C").

The "crystalline resin" means a resin that has a value of the aforementioned crystallinity index of 0.6 or more and less than 1.4, and preferably 0.8 or more and 1.2 or less.

- 10 The crystalline resin C is preferably a resin containing an aliphatic polyol as the alcohol component among the aforementioned resins. The preferred examples of the aliphatic polyol compound are the same as the examples described above.
- 15 The softening point of the resin C is preferably 100° C. or less, and more preferably 90° C. or less, from the standpoint of the low-temperature fusing property, and is preferably 60° C. or more, more preferably 70° C. or more, and further preferably 80° C. or more, from the standpoint of the high-temperature offset resistance.

20 The melting point of the resin C is preferably 100° C. or less, and more preferably 90° C. or less, from the standpoint of the low-temperature fusing property, and is preferably 60° C. or more, more preferably 70° C. or more, and further preferably 80° C. or more, from the standpoint of the high-temperature offset resistance.

25 The content of the resin C is preferably 1% by mass or more, more preferably 2% by mass or more, and further preferably 3% by mass or more, and is preferably 20% by mass or less, more preferably 15% by mass or less, and further preferably 8% by mass or less, based on the binder resin.

30 The total content of the polyester, the styrene resin, and the composite resin is preferably 80% by mass or more, more preferably 90% by mass or more, and further preferably 95% by mass or more, and is preferably 100% by mass or less, based on the binder resin.

## &lt;Charge Controlling Agent&gt;

35 The toner for electrophotography of the present invention preferably contains a charge controlling agent.

The combination use of the particular polyhydroxyamine compound and a charge controlling agent may provide a toner for electrophotography exhibiting a better charge rise property. While the reason therefor is not clear, one of the factors enhancing the charge rise property can be estimated that the particular polyhydroxyamine compound is adsorbed on the surface of the charge controlling agent, and the dispersion of the charge controlling agent is improved with the structure having high affinity to the binder resin.

40 The charge controlling agent is not particularly limited, and any of a positive charge controlling agent and a negative charge controlling agent may be contained.

45 Examples of the positive charge controlling agent include a nigrosine dye, such as "Nigrosine Base EX", "Oil Black BS", "Oil Black SO", "Bontron N-01", "Bontron N-04", "Bontron N-07", "Bontron N-09", and "Bontron N-11" (all produced by Orient Chemical Industries, Co., Ltd.); a triphenylmethane dye having a tertiary amine as a side chain, a quaternary ammonium salt compound, such as "Bontron P-51" (produced by Orient Chemical Industries, Co., Ltd.), cetyltrimethylammonium bromide, "Copy Charge PX VP435" (produced by Clariant AG); a polyamine resin, such as "AFP-B" (produced by Orient Chemical Industries, Co., Ltd.); an imidazole derivative, such as "PLZ-2001" and "PLZ-8001" (all produced by Shikoku Chemicals Corporation); and a styrene-acrylic resin, such as "FCA-701PT" (produced by Fujikura Kasei Co., Ltd.).

Examples of the negative charge controlling agent include a metal-containing azo dye, such as "Valifast Black 3804", "Bontron S-31", "Bontron S-32", "Bontron S-34", and "Bontron S-36" (all produced by Orient Chemical Industries, Co., Ltd.), and "Aizen Spilon Black THE" and "T-77" (all produced by Hodogaya Chemical Co., Ltd.); a metal compound of a benzilic acid, such as "LR-147" and "LR-297" (all produced by Japan Carlit Co., Ltd.), a metal compound of a salicylic acid compound, such as "Bontron E-81", "Bontron E-84", "Bontron E-88", and "Bontron E-304" (all produced by Orient Chemical Industries, Co., Ltd.), and "TN-105" (produced by Hodogaya Chemical Co., Ltd.); a copper phthalocyanine dye; a quaternary ammonium salt, such as "Copy Charge NX VP434" (produced by Clariant AG), a nitroimidazole derivative; and an organic metal compound.

Among the charge controlling agents, a negative charge controlling agent is preferred, and a metal compound of a benzilic acid compound and a metal compound of a salicylic acid compound are more preferred.

The content of the charge controlling agent is preferably 0.01 part by mass or more, and more preferably 0.2 part by mass or more, from the standpoint of the charge rise property of the toner, and is preferably 10 parts by mass or less, more preferably 5 parts by mass or less, further preferably 3 parts by mass or less, and still further preferably 2 parts by mass or less, from the same standpoint, per 100 parts by mass of the binder resin.

<Colorant>

The colorant may be any of dyes, pigments, and the like that have been used as a colorant for a toner, and examples thereof include carbon black, phthalocyanine blue, permanent brown FG, brilliant fast scarlet, pigment green B, rhodamine-B base, solvent red 49, solvent red 146, solvent blue 35, quinacridone, carmine 6B, and disazo yellow. The toner of the present invention may be any of a black toner and a color toner.

The content of the colorant is preferably 1 part by mass or more, and more preferably 2 parts by mass or more, and is preferably 40 parts by mass or less, more preferably 20 parts by mass or less, and further preferably 10 parts by mass or less, per 100 parts by mass of the binder resin, from the standpoint of enhancing the image density of the toner.

<Release Agent>

The toner for electrophotography may contain a release agent.

Examples of the release agent include polypropylene wax, polyethylene wax, and polypropylene-polyethylene copolymer wax; hydrocarbon wax, such as microcrystalline wax, paraffin wax, Fischer-Tropsch wax, and Sasol wax, and oxides thereof; ester wax, such as carnauba wax and montan wax, and deoxidized wax thereof, and fatty acid ester wax; a fatty acid amide compound, a fatty acid compound, a higher alcohol compound, and a fatty acid metal salt, and one kind or two or more kinds thereof may be used.

The melting point of the release agent is preferably 60° C. or more, and more preferably 70° C. or more, from the standpoint of the transferability of the toner, and is preferably 160° C. or less, and more preferably 140° C. or less, from the standpoint of the low-temperature fusing property.

The content of the release agent is preferably 0.5 part by mass or more, more preferably 1.0 part by mass or more, and further preferably 1.5 parts by mass or more, from the standpoint of the low-temperature fusing property and the offset resistance of the toner, and is preferably 10 parts by mass or less, more preferably 8 parts by mass or less, and

further preferably 7 parts by mass or less, from the standpoint of the dispersibility in the binder resin, per 100 parts by mass of the binder resin.

The raw material of the toner for electrophotography may further contain additives, such as magnetic powder, a fluidity enhancer, a conductivity controlling agent, a reinforcing filler, such as a fibrous substance, an antioxidant, an anti-aging agent, and a cleaning property enhancer.

The volume median diameter ( $D_{50}$ ) of the toner for electrophotography of the present invention is preferably 2  $\mu\text{m}$  or more, more preferably 3  $\mu\text{m}$  or more, and further preferably 4  $\mu\text{m}$  or more, and is preferably 20  $\mu\text{m}$  or less, more preferably 15  $\mu\text{m}$  or less, and further preferably 10  $\mu\text{m}$  or less.

[Process for Producing Toner for Electrophotography]

Examples of the process for producing a toner for electrophotography of the present invention include:

(1) a process including melt-kneading a toner raw material mixture containing a binder resin; and pulverizing a resulting melt-kneaded material, thereby producing a toner,

(2) a process including aggregating and fusing binder resin particles in a toner raw material mixture containing a dispersion liquid having a binder resin dispersed in an aqueous dispersion medium, so as to provide toner particles, thereby producing a toner, and

(3) a process including high-speed agitating a dispersion liquid having a binder resin dispersed in an aqueous medium, and a toner raw material, so as to provide toner particles, thereby producing a toner.

The polyhydroxyamine compound may be added in any of the process steps. The melt-kneading process (1) is preferred from the standpoint of enhancing the productivity of the toner and the standpoint of enhancing the fusing property of the toner. The toner may also be obtained by the aggregation and fusion process (2).

The time of addition in the process (1) is preferably the step of mixing the raw materials including the binder resin, from the standpoint of the dispersibility.

In the production of the toner by any of the aforementioned processes, the amount of the binder resin used is preferably 5% by mass or more, more preferably 30% by mass or more, further preferably 50% by mass or more, still further preferably 70% by mass or more, still more further preferably 80% by mass or more, and still more further preferably 90% by mass or more, and is preferably 100% by mass or less, and more preferably 99% by mass or less, based on the toner, from the standpoint of enhancing the storage stability of the toner and the fusing property of the toner.

(1) Melt-Kneading Process

In the melt-kneading process, it is preferred that a toner raw material mixture containing a binder resin, and the polyhydroxyamine compound represented by the formula (1) in an amount of 0.001 part by mass or more and 5.0 parts by mass or less per 100 parts by mass of the binder resin are melt-kneaded, and the resulting melt-kneaded material is pulverized, thereby producing the toner.

The process (1) preferably includes the following steps 1 and 2:

step 1: a step of melt-kneading a toner raw material mixture containing a binder resin, and the polyhydroxyamine compound represented by the formula (1) in an amount of 0.001 part by mass or more and 5.0 parts by mass or less per 100 parts by mass of the binder resin, and

step 2: a step of pulverizing and classifying the melt-kneaded material obtained in the step 1.

In the step 1, it is more preferred that a colorant is further melt-kneaded, and it is preferred that additional additives, such as a release agent and a charge controlling agent, are also melt-kneaded.

The melt-kneading may be performed with a known kneader, such as a closed kneader, a single screw or twin screw extruder, and an open roll kneader. An open roll kneader is preferably used since the additives, such as the colorant, the charge controlling agent, and the release agent, can be highly dispersed in the toner with high efficiency even without the use of repetition of kneading or the use of a dispersion assistant, and the open roll kneader is preferably equipped with a feeding port and a kneaded material discharging port along the axial direction of the roll.

It is preferred that the toner raw materials including the binder resin, the polyhydroxyamine compound, the colorant, the charge controlling agent, the release agent, and the like are mixed with a mixer, such as a Henschel mixer and a ball mill, in advance, and then supplied to the kneader.

The open roll kneader has a kneading part that is not closed but is open, and the kneading heat generated on kneading can be readily radiated. A continuous open roll kneader is preferably a kneader that is equipped with at least two rolls, and the continuous open roll kneader used in the present invention is a kneader that is equipped with two rolls different in circumferential velocity, i.e., two rolls including a high-rotation roll having a large circumferential velocity and a low-rotation roll having a small circumferential velocity. In the present invention, it is preferred that the high-rotation roll is a heating roll, and the low-rotation roll is a cooling roll, from the standpoint of enhancing the dispersibility of the colorant, the charge controlling agent, the releasing agent, and the like in the toner, the standpoint of decreasing the mechanical force on melt-kneading to suppress the heat generation, and the standpoint of decreasing the temperature on melt-kneading.

The temperature of the melt-kneading (i.e., the heating temperature in the roll) is preferably 20° C. or more, and more preferably 30° C. or more, and is preferably (the boiling point of the polyhydroxyamine compound under ordinary pressure-30° C.) or less, more specifically, preferably 150° C. or less, and more preferably 130° C. or less, from the standpoint of the dispersibility of the additives.

The temperature of the roll can be controlled, for example, by the temperature of the heat medium passing through the interior of the roll.

The circumferential velocity of rotation of the rolls for a co-rotation twin screw extruder is preferably 5 m/min or more, more preferably 10 m/min or more, and further preferably 20 m/min or more, and is preferably 50 m/min or less, more preferably 40 m/min or less, and further preferably 30 m/min or less, from the standpoint of enhancing the dispersibility of the colorant, the charge controlling agent, the release agent, and the like in the toner, and the standpoint of decreasing the mechanical force on melt-kneading to suppress the heat generation.

The circumferential velocity of the high-rotation roll is preferably 2 m/min or more, more preferably 10 m/min or more, and further preferably 25 m/min or more, and is preferably 100 m/min or less, more preferably 75 m/min or less, and further preferably 50 m/min or less, from the standpoint of enhancing the dispersibility of the release agent, the colorant, the charge controlling agent, and the like in the toner, the standpoint of decreasing the mechanical force on melt-kneading to suppress the heat generation, and the standpoint of enhancing the durability and the low-temperature fusing property of the toner.

The circumferential velocity of the low-rotation roll is preferably 1 m/min or more, more preferably 5 m/min or more, and further preferably 15 m/min or more, and is preferably 90 m/min or less, more preferably 60 m/min or less, and further preferably 30 m/min or less, from the same standpoint. The ratio of the circumferential velocities of the two rolls (low-rotation roll/high-rotation roll) is preferably from 1/10 to 9/10, and more preferably from 3/10 to 8/10.

The rolls are not particularly limited in structure, size, material, and the like, and the surfaces of the rolls may be any of a flat surface, a waved surface, an uneven surface, and the like, and preferably have plural spiral grooves formed thereon from the standpoint of increasing the kneading shear force to enhance the dispersibility of the colorant, the charge controlling agent, the release agent, and the like in the toner, and the standpoint of decreasing the mechanical force on melt-kneading to suppress the heat generation.

The melt-kneaded material obtained in the step 1 is cooled to such an extent that the material can be pulverized, and then supplied to the step 2.

In the step 2, the melt-kneaded material obtained in the step 1 is pulverized and classified.

The pulverizing step may be performed in multiple stages. For example, the resin kneaded material obtained by curing the melt-kneaded material may be coarsely pulverized to a size of approximately from 1 to 5 mm, and the finely pulverized to the target particle diameter.

The pulverizer used in the pulverizing step is not particularly limited, and examples of the pulverizer that may be preferably used for coarse pulverization include a hummer mill, an atomizer, and Rotoplex. Examples of the pulverizer that may be preferably used for fine pulverization include a fluidized bed jet mill, a collision plate jet mill, and a rotary mechanical mill. From the standpoint of the pulverization efficiency, a fluidized bed jet mill and a collision plate jet mill are preferably used, and a fluidized bed jet mill is more preferably used.

Examples of the classifier used for the classifying step include a rotor classifier, an airflow classifier, an inertial classifier, and a sieve classifier. The pulverized product that is removed in the classifying step due to the insufficient pulverization may be again supplied to the pulverizing step, and the pulverizing step and the classifying step may be repeated depending on necessity.

The process (1) may further include the following step 3: step 3: mixing the powder obtained through classification with an external additive.

Examples of the external additive include inorganic fine particles, such as hydrophobic silica, titanium oxide fine particles, alumina fine particles, cerium oxide fine particles, and carbon black, and polymer fine particles, such as polycarbonate, polymethyl methacrylate, and a silicone resin, and among these, hydrophobic silica is preferred.

In the case where the toner particles are subjected to a surface treatment with an external additive, the amount of the external additive added is preferably 0.1 part by mass or more, more preferably 0.5 part by mass or more, and further preferably 1.0 part by mass or more, and is preferably 5 parts by mass or less, more preferably 4 parts by mass or less, and further preferably 3 parts by mass or less, per 100 parts by mass of the toner particles.

In relation to the aforementioned embodiments, the present invention further relates to the toners for electrophotography, and the like shown below.

<1> A toner for electrophotography containing a binder resin, and a polyhydroxyamine compound represented by

the following formula (1) in an amount of 0.001 part by mass or more and 5.0 parts by mass or less per 100 parts by mass of the binder resin:



wherein  $\text{R}^1$  represents a hydrogen atom, an alkyl group having a number of carbon atoms of 1 or more and 5 or less, or a hydroxyalkyl group having a number of carbon atoms of 1 or more and 5 or less;  $\text{R}^2$  represents a hydrogen atom, an alkyl group having a number of carbon atoms of 1 or more and 6 or less, or a hydroxyalkyl group having a number of carbon atoms of 1 or more and 5 or less; and  $\text{R}^3$  and  $\text{R}^4$  each represent an alkanediyl group having a number of carbon atoms of 1 or more and 5 or less, provided that  $\text{R}^3$  and  $\text{R}^4$  may be the same as or different from each other.

<2> The toner for electrophotography according to the item <1>, wherein the polyhydroxyamine compound is at least one selected from 2-amino-1,3-propanediol, 2-amino-2-methyl-1,3-propanediol, 2-amino-2-ethyl-1,3-propanediol, 2-amino-2-hydroxymethyl-1,3-propanediol, and 2-amino-2-hydroxyethyl-1,3-propanediol.

<3> The toner for electrophotography according to the item <1> or <2>, wherein the polyhydroxyamine compound is 2-amino-2-hydroxymethyl-1,3-propanediol.

<4> The toner for electrophotography according to any one of the items <1> to <3>, wherein the content of the polyhydroxyamine compound is 0.001 part by mass or more, preferably 0.01 part by mass or more, more preferably 0.03 part by mass or more, further preferably 0.01 part by mass or more, and still further preferably 0.3 part by mass or more, and is 5.0 parts by mass or less, preferably 4.0 parts by mass or less, and more preferably 3.0 parts by mass or less per 100 parts by mass of the binder resin.

<5> The toner for electrophotography according to any one of the items <1> to <4>, further containing a charge controlling agent, preferably a negative charge controlling agent, and more preferably a metal compound of a benzilic acid, or a metal compound of a salicylic acid compound.

<6> The toner for electrophotography according to any one of the items <1> to <5>, wherein the content of the charge controlling agent is preferably 0.01 part by mass or more, and more preferably 0.2 part by mass or more, and is preferably 10 parts by mass or less, more preferably 5 parts by mass or less, further preferably 3 parts by mass or less, and still further preferably 2 parts by mass or less, per 100 parts by mass of the binder resin.

<7> The toner for electrophotography according to any one of the items <1> to <6>, wherein the binder resin is a polycondensation resin, such as a polyester and a polyamide, a styrene resin, such as a styrene resin and a styrene-acrylic resin, an epoxy resin, a polycarbonate, a polyurethane, or a composite resin of these resins.

<8> The toner for electrophotography according to any one of the items <1> to <7>, wherein the binder resin preferably contains at least one selected from a resin having a polyester moiety obtained through polycondensation of an alcohol component and a carboxylic acid component, and a styrene resin, more preferably contains at least one selected from a urethane-modified polyester resin, a polyester, a styrene resin, and a composite resin having a polyester

segment and a styrene resin segment, and further preferably contains at least one selected from a polyester, a styrene resin, and a composite resin having a polyester segment and a styrene resin segment.

5 <9> The toner for electrophotography according to any one of the items <1> to <8>, containing at least one selected from a polyester and a composite resin having a polyester segment as the binder resin.

10 <10> The toner for electrophotography according to the item <9>, wherein the alcohol component of the polyester contains an alkylene oxide adduct of bisphenol A.

15 <11> The toner for electrophotography according to any one of the items <1> to <10>, wherein the number average molecular weight of the binder resin is 1,000 or more, and is 7,000 or less, preferably 6,000 or less, and more preferably 5,500 or less.

20 <12> The toner for electrophotography according to any one of the items <1> to <11>, wherein the softening point of the binder resin is 90° C. or more, preferably 95° C. or more, and more preferably 100° C. or more, and is 160° C. or less, preferably 150° C. or less, more preferably 145° C. or less, and further preferably 140° C. or less.

25 <13> The toner for electrophotography according to any one of the items <1> to <12>, wherein the glass transition temperature of the binder resin is 45° C. or more, preferably 50° C. or more, and more preferably 55° C. or more, and is 80° C. or less, preferably 75° C. or less, more preferably 70° C. or less, and further preferably 65° C. or less.

30 <14> The toner for electrophotography according to any one of the items <1> to <13>, wherein the acid value of the binder resin is 40 mgKOH/g or less, preferably 30 mgKOH/g or less, and more preferably 20 mgKOH/g or less, and is 1 mgKOH/g or more, and preferably 2 mgKOH/g or more.

35 <15> The toner for electrophotography according to any one of the items <1> to <14>, wherein the binder resin contains an amorphous polyester.

40 <16> The toner for electrophotography according to any one of the items <1> to <15>, wherein the binder resin contains a composite resin having a polyester segment and a styrene resin segment.

45 <17> The toner for electrophotography according to any one of the items <1> to <16>, wherein the composite resin is a resin obtained through polymerization of (i) a raw material monomer of a polyester segment containing an alcohol component containing an alkylene oxide adduct of bisphenol A, and a carboxylic acid component containing an aromatic dicarboxylic acid, (ii) a raw material monomer of a styrene resin segment, and (iii) a bireactive monomer capable of reacting with both the raw material monomer of the polyester segment and the raw material monomer of the styrene resin segment.

50 <18> The toner for electrophotography according to any one of the items <1> to <17>, wherein the bireactive monomer is a compound that has in the molecule thereof at least one functional group selected from a hydroxy group, a carboxy group, an epoxy group, a primary amino group, and a secondary amino group, preferably at least one functional group selected from a hydroxy group and a carboxy group, and more preferably a carboxy group and an ethylenic unsaturated bond, and is further preferably at least one selected from acrylic acid, methacrylic acid, fumaric acid, maleic acid, and maleic anhydride.

55 <19> The toner for electrophotography according to any one of the items <1> to <18>, wherein the binder resin contains a urethane-modified polyester resin obtained

through reaction of one kind or two or more kinds of a polyester and a polyisocyanate compound.

<20> A process for producing a toner for electrophotography, including: melt-kneading a toner raw material mixture containing a binder resin, and a polyhydroxyamine compound represented by the following formula (1) in an amount of 0.001 part by mass or more and 5.0 parts by mass or less per 100 parts by mass of the binder resin; and pulverizing a resulting melt-kneaded material:



wherein  $\text{R}^1$  represents a hydrogen atom, an alkyl group having a number of carbon atoms of 1 or more and 5 or less, or a hydroxyalkyl group having a number of carbon atoms of 1 or more and 5 or less;  $\text{R}^2$  represents a hydrogen atom, an alkyl group having a number of carbon atoms of 1 or more and 6 or less, or a hydroxyalkyl group having a number of carbon atoms of 1 or more and 5 or less; and  $\text{R}^3$  and  $\text{R}^4$  each represent an alkanediyl group having a number of carbon atoms of 1 or more and 5 or less, provided that  $\text{R}^3$  and  $\text{R}^4$  may be the same as or different from each other.

<21> The process for producing a toner for electrophotography according to the item <20>, wherein the melt-kneading is performed with an open roll kneader.

<22> The process for producing a toner for electrophotography according to the item <20> or <21>, wherein the temperature of the melt-kneading is preferably 20° C. or more, and more preferably 30° C. or more, and is preferably (the boiling point of the polyhydroxyamine compound under ordinary pressure-30° C.) or less, more specifically, preferably 150° C. or less, and more preferably 130° C. or less.

<23> Use of a polyhydroxyamine compound represented by the formula (1) for a toner for electrophotography.

<24> Use of a polyhydroxyamine compound represented by the formula (1) for enhancing a charge rise property of a toner for electrophotography.

## EXAMPLES

The property values of the resins and the like were measured and evaluated in the following manners.

### [Acid Value of Resin]

The acid value of the resin was measured according to the method of JIS K0070, provided that only the measurement solvent was changed from a mixed solvent of ethanol and ether defined in JIS K0070 to a mixed solvent of acetone and toluene (acetone/toluene=1/1 (volume ratio)).

### [Softening Point and Glass Transition Temperature of Resin]

#### (1) Softening Point

By using a flow tester, "CFT-500D" (produced by Shimadzu Corporation), 1 g of a specimen was extruded through a nozzle having a diameter of 1 mm and a length of 1 mm under application of a load of 1.96 MPa thereto with a plunger while heating the specimen at a temperature rising rate of 6° C./min. The descent amount of the plunger of the flow tester was plotted with respect to the temperature, and the temperature, at which a half amount of the specimen flowed out, was designated as the softening point.

### (2) Highest Endothermic Peak Temperature of Resin

By using a differential scanning calorimeter, "Q-100" (produced by TA Instruments Japan Inc.), a specimen was cooled from room temperature (20° C.) to 0° C. at a temperature decreasing rate of 10° C./min and held for 1 minute. Thereafter, the specimen was measured while heating to 180° C. at a temperature rising rate of 10° C./min. The temperature of the peak that had the highest temperature among the endothermic peaks observed was designated as the highest endothermic peak temperature.

### (3) Glass Transition Temperature

By using a differential scanning calorimeter, "Q-100" (produced by TA Instruments Japan Inc.), from 0.01 to 0.02 g of a specimen weighed on an aluminum pan was heated to 200° C. and then cooled from that temperature to 0° C. at a temperature decreasing rate of 10° C./min. The specimen was then measured while heating to 150° C. at a temperature rising rate of 10° C./min and measured. The intersection point of the extended line of the base line below the highest endothermic peak temperature and the tangential line showing the maximum gradient between the rising part of the peak and the apex of the peak was designated as the glass transition temperature.

### (4) Number Average Molecular Weight and Weight Average Molecular Weight of Resin

The molecular weight distribution was measured by the gel permeation chromatography (GPC) method according to the following manner, from which the number average molecular weight  $M_n$  and the weight average molecular weight  $M_w$  of the resin were obtained.

#### (4-1) Preparation of Specimen Solution

The resin was dissolved in chloroform to make a concentration of 0.5 g/100 mL. The solution was filtered with a fluorine resin filter having a pore size of 2 μm ("FP-200", a trade name, produced by Sumitomo Electric Industries, Ltd.) to remove insoluble components, and thus a specimen solution was prepared.

#### (4-2) Measurement of Molecular Weight

In the device shown below, chloroform as an eluent was flowed through a flow rate of 1 mL/min, and the column was stabilized in a thermostat chamber at 40° C. 100 μL of the specimen solution was injected thereto and measured. The molecular weight of the specimen was calculated based on the calibration line having been prepared in advance. The calibration line used herein was prepared by using the monodisperse polystyrene samples ( $2.63 \times 10^3$ ,  $2.06 \times 10^4$ , and  $1.02 \times 10^5$ , produced by Tosoh Corporation, and  $2.10 \times 10^3$ ,  $7.00 \times 10^3$ , and  $5.04 \times 10^4$ , produced by GL Sciences, Inc.) as the standard sample.

Measuring device: "CO-8010" (produced by Tosoh Corporation) Analysis columns: "GMH<sub>XZ</sub>" and "G3000H<sub>XZ</sub>" (all produced by Tosoh Corporation)

#### [Volume Median Particle Diameter ( $D_{50}$ ) of Toner]

The volume median particle diameter ( $D_{50}$ ) of the toner was measured in the following manner.

Measuring device: Coulter Multisizer II (produced by Beckman Coulter Inc.)

Aperture diameter: 50 μm

Analysis software: Coulter Multisizer AccuComp, ver. 1.19 (produced by Beckman Coulter Inc.)

Electrolytic solution: Isoton II (produced by Beckman Coulter Inc.)

Dispersion liquid: Emulgen 109P (produced by Kao Corporation, polyoxyethylene lauryl ether, HLB: 13.6) 5% electrolytic solution

Dispersion condition: 10 mg of a measurement specimen was added to 5 mL of the dispersion liquid and dispersed with an ultrasonic dispersing device for 1 minute, and 25 mL

of the electrolytic solution was then further added thereto and dispersed with an ultrasonic dispersing device for 1 minute.

Measurement condition: 100 mL of the electrolytic solution and the dispersion liquid were placed in a beaker, 30,000 particles were measured under a concentration capable of measuring 30,000 particles within 20 seconds, and the volume median particle diameter ( $D_{50}$ ) was obtained from the particle size distribution.

[Evaluation: Charge Rise]

At a temperature of 25°C. and a relative humidity of 50%, 0.6 g of the toner and 19.4 g of a silicone-ferrite carrier (produced by Kanto Denka Kogyo Co., Ltd., average particle diameter: 90  $\mu\text{m}$ ) were placed in a resin bottle having a capacity of 50 mL, and mixed with a ball mill at 250 r/min, and the charge amount was measured with a Q/M meter (produced by Epping GmbH).

After mixing for a prescribed period of time, a prescribed amount of a developer was placed in the cell accompanied by the Q/M meter, and only the toner was sucked through a sieve having an aperture of 32  $\mu\text{m}$  (formed of stainless steel, twill weave, wire diameter: 0.0035 mm) for 90 seconds. The change of voltage occurring at this time on the carrier was monitored, and the value of (total amount of electricity ( $\mu\text{C}$ ) after 90 seconds/amount (g) of toner sucked) was designated as the charge amount ( $\mu\text{C/g}$ ). The ratio of the charge amount after mixing for 60 seconds and the charge amount after mixing for 600 seconds (charge amount after mixing for 60 seconds/charge amount after mixing for 600 seconds) was calculated to evaluate the charge rise characteristics.

[Evaluation: Odor Suppression Capability]

5 g of the toner obtained in Example or Comparative Example was heated on a hot plate at 200°C. for 5 minutes, and the odor thereof was evaluated by 10 persons with ranks 1 to 4 (1: extremely offensive odor, 2: offensive odor, 3: substantially no odor, 4: no odor). The average values of the evaluation results of the 10 persons are shown in the table.

Production Examples of Resin

Production Example H1 (Resin H-1)

The raw material monomers of a polyester except for fumaric acid and trimellitic anhydride, and the esterification catalyst shown in Table 1 were placed in a four-neck flask having a capacity of 10 L equipped with a thermometer, a stainless steel stirrer, a fractionating column, a dehydration tube, a cooling tube, and a nitrogen introduction tube, and heated to 235°C. with a mantle heater in a nitrogen atmosphere, the reaction was performed for 7 hours, it was confirmed that the reaction rate reached 80% or more, and the reaction was performed at 20 kPa for 1 hour.

Thereafter, after cooling to 160°C., a mixture of styrene and 2-ethylhexyl acrylate as the raw material monomer of the segment (A2) (styrene resin), acrylic acid as the bireactive monomer, and dibutyl peroxide as the polymerization initiator, shown in Table 1, was added dropwise thereto over 1 hour. After completing the dropwise addition, the reaction mixture was held at 160°C. for 1 hour, then the temperature was increased to 200°C., the reaction was performed at 8 kPa for 0.5 hour, then fumaric acid and trimellitic anhydride were added, the reaction was performed under ordinary pressure for 1 hour, then the temperature was increased to 210°C., the reaction was performed for 1 hour, and then the reaction was performed at 8 kPa until the target softening point was obtained, thereby providing a resin H-1. The

reaction rate herein means a value of (amount of reaction water formed/theoretical amount of water formed)  $\times 100$  (hereinafter the same).

5 Production Example H2 (Resin H-2)

The raw material monomers except for fumaric acid and trimellitic anhydride, and the esterification catalyst shown in Table 1 were placed in a four-neck flask having a capacity of 10 L equipped with a thermometer, a stainless steel stirrer, a fractionating column, a dehydration tube, a cooling tube, and a nitrogen introduction tube, and heated to 235°C. with a mantle heater in a nitrogen atmosphere, the reaction was performed for 7 hours, it was confirmed that the reaction rate reached 80% or more, the temperature was decreased to 190°C., fumaric acid and trimellitic anhydride were added, the temperature was increased to 210°C. at a rate of 10°C./h, then the reaction was performed under ordinary pressure for 1 hour, and then the reaction was performed at 8 kPa until the target softening point was obtained, thereby providing a resin H-2.

20 Production Example H3 (Resin H-3)

The raw material monomers except for trimellitic anhydride, and the esterification catalyst shown in Table 1 were placed in a four-neck flask having a capacity of 10 L equipped with a thermometer, a stainless steel stirrer, a fractionating column, a dehydration tube, a cooling tube, and a nitrogen introduction tube, and heated to 235°C. with a mantle heater in a nitrogen atmosphere, the reaction was performed for 7 hours, it was confirmed that the reaction rate reached 80% or more, the temperature was decreased to 210°C., trimellitic anhydride was added, the reaction was performed under ordinary pressure for 1 hour, and then the reaction was performed at 8 kPa until the target softening point was obtained, thereby providing a resin H-3.

25 Production Example H4 (Resin H-4)

The raw material monomers except for trimellitic anhydride, and the esterification catalyst shown in Table 1 were placed in a four-neck flask having a capacity of 10 L equipped with a thermometer, a stainless steel stirrer, a fractionating column, a dehydration tube, a cooling tube, and a nitrogen introduction tube, and heated to 185°C. with a mantle heater in a nitrogen atmosphere, the reaction was performed for 5 hours, the temperature was increased to 220°C. at 10°C./h, it was confirmed that the reaction rate reached 80% or more at 220°C., the temperature was decreased to 210°C., trimellitic anhydride was added, the reaction was performed under ordinary pressure for 1 hour, and then the reaction was performed at 8 kPa until the target softening point was obtained, thereby providing a resin H-4.

30 Production Example H5 (Resin H-5)

35 60 1,000 g of xylene was placed in a four-neck flask having a capacity of 5 L equipped with a nitrogen introduction tube, a dehydration tube, a stirrer, and a thermocouple, and under stirring at 125°C. in a nitrogen atmosphere, a mixture of the raw materials shown in Table 1 was added dropwise thereto from a dropping funnel over 2 hours. The temperature was held at 125°C. for 1 hour, then refluxing was performed at 150°C. for 1 hour, the reaction system was held at 200°C.

and 8.0 kPa, and xylene was distilled off over 2 hours, thereby providing a resin H-5.

#### Production Example H6 (Resin H-6)

The raw material monomers except for fumaric acid and trimellitic anhydride, and the esterification catalyst shown in Table 1 were placed in a four-neck flask having a capacity of 10 L equipped with a thermometer, a stainless steel stirrer, a fractionating column, a dehydration tube, a cooling tube, and a nitrogen introduction tube, and heated to 235° C. with

a mantle heater in a nitrogen atmosphere, the reaction was performed for 7 hours, it was confirmed that the reaction rate reached 80% or more, the temperature was decreased to 190° C., fumaric acid and trimellitic anhydride were added, 5 the temperature was increased to 210° C. at a rate of 10° C./h, and then the reaction was performed under ordinary pressure for 1 hour. Thereafter, the reaction was performed at 8 kPa to provide a polyester. 2 parts by mass of isophorone diisocyanate was added to 100 parts by mass of the resulting 10 resin, and the reaction was performed at 180° C. for 30 minutes.

TABLE 1

| Production Example                                              |                                      |                       |                       |                       |                    |                 |                    |      |
|-----------------------------------------------------------------|--------------------------------------|-----------------------|-----------------------|-----------------------|--------------------|-----------------|--------------------|------|
|                                                                 |                                      | Production Example H1 | Production Example H2 | Production Example H3 | Resin              |                 |                    |      |
|                                                                 |                                      | Resin H-1             |                       | Resin H-2             |                    | Resin H-3       |                    |      |
|                                                                 |                                      | part by mol *1        | charged amount (g)    | part by mol *1        | charged amount (g) | part by mol *1  | charged amount (g) |      |
| Raw material monomer of component                               | Alcohol                              | BPA-PO *5             | 70                    | 3430                  | 50                 | 2450            | 70                 | 3430 |
|                                                                 |                                      | BPA-EO *6             | 30                    | 1365                  | 50                 | 2275            | 30                 | 1365 |
| polyester and polyester segment                                 | 1,2-Propanediol                      |                       |                       |                       |                    |                 |                    |      |
|                                                                 | 1,4-Butanediol                       |                       |                       |                       |                    |                 |                    |      |
| Acid component                                                  | Terephthalic acid                    | 50                    | 1162                  | 50                    | 1162               | 60              | 1394               |      |
|                                                                 | Fumaric acid                         | 10                    | 162                   | 10                    | 162                |                 |                    |      |
| Esterification catalyst                                         | Dodecenylsuccinic anhydride          |                       |                       |                       |                    | 15              | 563                |      |
|                                                                 | Trimellitic anhydride                | 15                    | 403                   | 20                    | 538                | 10              | 269                |      |
|                                                                 | Tin(II) 2-ethylhexanoate (% by mass) | 0.5                   | 33                    | 0.5                   | 33                 | 0.5             | 35                 |      |
| Promoter                                                        | Gallic acid monohydrate (% by mass)  | 0.03                  | 2.0                   | 0.03                  | 2.0                | 0.03            | 2.1                |      |
| Bireactive monomer                                              | Acrylic acid                         | 6                     | 60.5                  |                       |                    |                 |                    |      |
| Polyisocyanate compound Isophorone diisocyanate                 |                                      |                       |                       |                       |                    |                 |                    |      |
|                                                                 |                                      | part by mass *2       | charged amount (g)    | part by mass *2       | charged amount (g) | part by mass *2 | charged amount (g) |      |
| Raw material monomer of styrene resin and styrene resin segment | Styrene                              |                       |                       |                       |                    |                 |                    |      |
|                                                                 | 2-Ethylhexyl acrylate                | 84                    | 1382                  |                       |                    |                 |                    |      |
|                                                                 | Butyl methacrylate                   | 16                    | 263                   |                       |                    |                 |                    |      |
| Polymerization initiator                                        | Dibutyl peroxide                     | part by mass *3       | charged amount (g)    | part by mass *3       | charged amount (g) | part by mass *3 | charged amount (g) |      |
|                                                                 | Dicumyl peroxide                     |                       |                       |                       |                    |                 |                    |      |
| Polyester segment/acrylic resin segment ratio                   |                                      |                       |                       |                       |                    |                 |                    |      |
| Properties of resin                                             | Acid/alcohol ratio of polyester      |                       | 80/20                 |                       |                    |                 |                    |      |
|                                                                 | Acid value (mgKOH/g)                 |                       | 0.855                 |                       | 0.900              |                 | 0.900              |      |
|                                                                 | Number average molecular weight (Mn) |                       | 23.6                  |                       | 18.7               |                 | 23.6               |      |
|                                                                 | Softening point (° C.)               |                       | 4200                  |                       | 4900               |                 | 4500               |      |
|                                                                 | Glass transition temperature (° C.)  |                       | 133.5                 |                       | 135.9              |                 | 136.4              |      |
| Crystallinity index                                             |                                      |                       |                       |                       |                    |                 |                    |      |
|                                                                 |                                      | % by mass *4          | charged amount (g)    | % by mass *4          | charged amount (g) | % by mass *4    | charged amount (g) |      |
| Polymerization initiator                                        | Dibutyl peroxide                     | 6                     | 99                    |                       |                    |                 |                    |      |
|                                                                 | Dicumyl peroxide                     |                       |                       |                       |                    |                 |                    |      |

TABLE 1-continued

|                                                                 |                                                                                                                                                      | Production Example                                                                                                                                       |                                       |                             |                                       |                       |                                           |                                                  |
|-----------------------------------------------------------------|------------------------------------------------------------------------------------------------------------------------------------------------------|----------------------------------------------------------------------------------------------------------------------------------------------------------|---------------------------------------|-----------------------------|---------------------------------------|-----------------------|-------------------------------------------|--------------------------------------------------|
|                                                                 |                                                                                                                                                      | Production Example H4                                                                                                                                    |                                       | Production Example H5 Resin |                                       | Production Example H6 |                                           |                                                  |
|                                                                 |                                                                                                                                                      | Resin H-4                                                                                                                                                |                                       | Resin H-5                   |                                       | Resin H-6             |                                           |                                                  |
|                                                                 |                                                                                                                                                      | part by mol *1                                                                                                                                           | charged amount (g)                    | part by mol *1              | charged amount (g)                    | part by mol *1        | charged amount (g)                        |                                                  |
| Raw material monomer of polyester and polyester segment         | Alcohol component                                                                                                                                    | BPA-PO *5<br>BPA-EO *6<br>1,2-Propanediol<br>1,4-Butanediol<br>Terephthalic acid<br>Fumaric acid<br>Dodecenylsuccinic anhydride<br>Trimellitic anhydride |                                       | 70<br>30<br>65<br>15        | 745<br>378<br>1511<br>403             |                       | 50<br>50<br>60<br>10<br>10<br>0.5<br>0.03 | 2450<br>2275<br>1394.4<br>162<br>269<br>0<br>0.0 |
| Esterification catalyst                                         | Tin(II) 2-ethylhexanoate (% by mass)                                                                                                                 | 0.5                                                                                                                                                      | 15                                    |                             |                                       | 0.5                   | 0                                         |                                                  |
| Promoter                                                        | Gallic acid monohydrate (% by mass)                                                                                                                  | 0.03                                                                                                                                                     | 0.9                                   |                             |                                       | 0.03                  | 0.0                                       |                                                  |
| Bireactive monomer                                              | Acrylic acid                                                                                                                                         |                                                                                                                                                          |                                       |                             |                                       |                       |                                           |                                                  |
| Polyisocyanate compound                                         | Isophorone diisocyanate                                                                                                                              |                                                                                                                                                          |                                       | part by mass *2             | charged amount (g)                    | part by mass *2       | charged amount (g)                        |                                                  |
| Raw material monomer of styrene resin and styrene resin segment | Styrene<br>2-Ethylhexyl acrylate<br>Butyl methacrylate                                                                                               |                                                                                                                                                          |                                       | 80<br>20                    | 1600<br>400                           |                       | 2<br>131                                  |                                                  |
| Polymerization initiator                                        | Dibutyl peroxide<br>Dicumyl peroxide                                                                                                                 |                                                                                                                                                          |                                       | % by mass *4                | charged amount (g)                    | % by mass *4          | charged amount (g)                        |                                                  |
| Polyester segment/acrylic resin segment ratio                   |                                                                                                                                                      |                                                                                                                                                          |                                       | 2                           | 40                                    |                       |                                           |                                                  |
| Acid/alcohol ratio of polyester                                 |                                                                                                                                                      |                                                                                                                                                          | 0.875                                 |                             |                                       |                       | 0.850                                     |                                                  |
| Properties of resin                                             | Acid value (mgKOH/g)<br>Number average molecular weight (Mn)<br>Softening point (° C.)<br>Glass transition temperature (° C.)<br>Crystallinity index |                                                                                                                                                          | 14.3<br>5200<br>132.4<br>57.6<br>2.18 |                             | 5200<br>138.5<br>60.2<br>59.3<br>2.12 |                       | 15.3<br>5500<br>140.2<br>59.3<br>2.21     |                                                  |

\*1 molar number per 100 moles of total amount of alcohol component

\*2 part by mass per 100 parts by mass of total amount of alcohol component and acid component

\*3 part by mass per 100 parts by mass of total amount of raw material monomer of styrene resin segment

\*4 % by mass based on total amount of raw material monomer of styrene resin segment

\*5 BPA-PO: polyoxypropylene(2,2)-2,2-bis 4-hydroxyphenyl)propane

\*6 BPA-EO: polyoxyethylene(2,0)-2,2-bis(4-hydroxyphenyl)propane

## Production Example L1 (Resin L-1)

The raw material monomers except for trimellitic anhydride, and the esterification catalyst shown in Table 2 were placed in a four-neck flask having a capacity of 10 L equipped with a thermometer, a stainless steel stirrer, a fractionating column, a dehydration tube, a cooling tube, and a nitrogen introduction tube, and heated to 235° C. with a mantle heater in a nitrogen atmosphere, the reaction was performed for 10 hours, it was confirmed that the reaction rate reached 80% or more, trimellitic anhydride was added, and the reaction was performed at 8 kPa until the target softening point was obtained, thereby providing a resin L-1.

## Production Example L2 (Resin L-2)

55 The raw material monomers of a polyester, the esterification catalyst, and the promoter shown in Table 2 were placed in a four-neck flask having a capacity of 10 L equipped with a thermometer, a stainless steel stirrer, a fractionating column, a dehydration tube, a cooling tube, 60 and a nitrogen introduction tube, and heated to 160° C. with a mantle heater in a nitrogen atmosphere, and a mixture of styrene and 2-ethylhexyl acrylate as the raw material monomers of a vinyl resin, acrylic acid as the bireactive monomer, and dibutyl peroxide as the polymerization initiator, shown in Table 2, was added dropwise thereto over 1 hour. After completing the dropwise addition, the reaction mixture was held at 160° C. for 1 hour, then the temperature was

increased to 235° C., the reaction was performed for 10 hours, it was confirmed that the reaction rate reached 80% or more, and the reaction was performed at 8 kPa until the target softening point was obtained, thereby providing a resin L-2.

## Production Example L3 (Resin L-3)

1,000 g of xylene was placed in a four-neck flask having a capacity of 5 L equipped with a nitrogen introduction tube, a dehydration tube, a stirrer, and a thermocouple, and under stirring at 135° C. in a nitrogen atmosphere, a mixture of the raw materials shown in Table 2 was added dropwise thereto from a dropping funnel over 2 hours. The temperature was held at 135° C. for 1 hour, then refluxing was performed at 150° C. for 1 hour, the reaction system was held at 200° C. and 8.0 kPa, and xylene was distilled off over 2 hours, thereby providing a resin L-3.

## Production Example L4 (Resin L-4)

The raw material monomers except for trimellitic anhydride, and the esterification catalyst shown in Table 2 were placed in a four-neck flask having a capacity of 10 L equipped with a thermometer, a stainless steel stirrer, a fractionating column, a dehydration tube, a cooling tube, and a nitrogen introduction tube, and heated to 235° C. with 5 a mantle heater in a nitrogen atmosphere, the reaction was performed for 10 hours, it was confirmed that the reaction rate reached 80% or more, trimellitic anhydride was added, and the reaction was performed at 8 kPa until the target softening point was obtained, thereby providing a resin L-1. 10 2 parts by mass of isophorone diisocyanate was added to 100 parts by mass of the resulting resin, and the reaction was performed at 180° C. for 30 minutes.

TABLE 2

|                                                                 | Production Example                   |                    |                       |                    |                       |                    |                       |                    |
|-----------------------------------------------------------------|--------------------------------------|--------------------|-----------------------|--------------------|-----------------------|--------------------|-----------------------|--------------------|
|                                                                 | Production Example L1                |                    | Production Example L2 |                    | Production Example L3 |                    | Production Example L4 |                    |
|                                                                 | Resin L-1                            |                    | Resin L-2             |                    | Resin L-3             |                    | Resin L-4             |                    |
|                                                                 | part by mol *1                       | charged amount (g) | part by mol *1        | charged amount (g) | part by mol *1        | charged amount (g) | part by mol *1        | charged amount (g) |
| Raw material monomer of component                               | Alcohol BPA-PO *5                    | 80                 | 3920                  | 20                 | 980                   |                    | 50                    | 2450               |
| polyester and polyester component                               | BPA-EO *6                            | 20                 | 910                   | 80                 | 3640                  |                    | 50                    | 2275               |
| segment                                                         | Terephthalic acid                    | 80                 | 1859                  | 92                 | 2138                  |                    | 75                    | 1743               |
| Esterification catalyst                                         | Trimellitic anhydride                | 5                  | 134                   |                    |                       |                    | 10                    | 269                |
| Promoter                                                        | Tin(II) 2-ethylhexanoate (% by mass) | 0.5                | 34                    | 0.5                | 34                    |                    | 0.5                   | 34                 |
| Bireactive monomer                                              | Gallic acid monohydrate (% by mass)  | 0.03               | 2.0                   | 0.03               | 2.0                   |                    | 0.03                  | 2.0                |
|                                                                 | Acrylic acid                         |                    |                       | 6                  | 60                    |                    |                       |                    |
|                                                                 | part by mass *2                      | charged amount (g) | part by mass *2       | charged amount (g) | part by mass *2       | charged amount (g) | part by mass *2       | charged amount (g) |
| Polyisocyanate compound                                         | Isophorone diisocyanate              |                    |                       |                    |                       |                    | 2                     | 136.5              |
|                                                                 | part by mass *3                      | charged amount (g) | part by mass *3       | charged amount (g) | part by mass *3       | charged amount (g) | part by mass *3       | charged amount (g) |
| Raw material monomer of styrene resin and styrene resin segment | Styrene                              |                    | 84                    | 1432               | 70                    | 1400               |                       |                    |
|                                                                 | 2-Ethylhexyl acrylate                |                    | 16                    | 273                |                       |                    |                       |                    |
|                                                                 | Butyl methacrylate                   |                    |                       |                    | 30                    | 600                |                       |                    |
|                                                                 | % by mass *4                         | charged amount (g) | % by mass *4          | charged amount (g) | % by mass *4          | charged amount (g) | % by mass *4          | charged amount (g) |
| Polymerization initiator                                        | Dibutyl peroxide                     |                    | 4                     | 68                 |                       |                    |                       |                    |
|                                                                 | Dicumyl peroxide                     |                    |                       |                    | 4                     | 80                 |                       |                    |
| Polyester segment/acrylic resin segment ratio                   |                                      |                    |                       | 80/20              |                       |                    |                       |                    |
| Acid/alcohol ratio of polyester                                 |                                      | 0.875              |                       | 0.950              |                       |                    |                       | 0.900              |
| Properties of resin                                             | Acid value (mg KOH/g)                | 14.3               |                       | 13.6               |                       |                    |                       | 14.3               |
|                                                                 | Number average molecular weight (Mn) | 2200               |                       | 2300               |                       | 3400               |                       | 2200               |
|                                                                 | Softening point (° C.)               | 101.3              |                       | 103.2              |                       | 103.2              |                       | 106.3              |
|                                                                 | Glass transition temperature (° C.)  | 60.3               |                       | 55.7               |                       | 52.6               |                       | 58.4               |
|                                                                 | Crystallinity index                  | 1.56               |                       | 1.71               |                       | 1.83               |                       | 1.70               |

\*1 molar number per 100 moles of total amount of alcohol component

\*2 part by mass per 100 parts by mass of total amount of alcohol component and acid component

\*3 part by mass per 100 parts by mass of total amount of raw material monomer of styrene resin segment

\*4 % by mass based on total amount of raw material monomer of styrene resin segment

\*5 BPA-PO: polyoxypropylene(2,2)-2,2-bis(4-hydroxyphenyl)propane

\*6 BPA-EO: polyoxyethylene(2,0)-2,2-bis(4-hydroxyphenyl)propane

## Production Examples C1 and C2 (Resins C-1 and C-2)

The raw material monomers and the esterification catalyst shown in Table 3 were placed in a four-neck flask having a capacity of 10 L equipped with a thermometer, a stainless steel stirrer, a fractionating column, a dehydration tube, and a cooling tube, and a nitrogen introduction tube, and heated to 140° C. with a mantle heater in a nitrogen atmosphere, the reaction was performed 5 hours, the temperature was increased to 200° C. at 10° C./h, it was confirmed that the reaction rate reached 80% or more at 200° C., and the reaction was performed at 8 kPa until the target softening point was obtained, thereby providing a resin C-1 (crystalline polyester). Resin C-2 (crystalline polyester) was obtained in the same manner.

of 43 mm. The rotation speed of the roll was 200 r/min, the heating temperature inside the roll was 120° C., the supplying rate of the mixture was 10 kg/hr, and the average retention time thereof was approximately 18 seconds. The resulting kneaded material was rolled and cooled with a cooling roller, and powder having a volume median particle diameter ( $D_{50}$ ) of 6.5  $\mu\text{m}$  was obtained with a jet mil.

To 100 parts by mass of the resulting powder, 1.0 part by mass of "Aerosil R-972" (hydrophobic silica, produced by Nippon Aerosil Co., Ltd., average particle diameter: 16 nm) and 1.0 part by mass of "SI-Y" (hydrophobic silica, produced by Nippon Aerosil Co., Ltd., average particle diameter: 40 nm) as external additives were added and mixed with a Henschel mixer at 3,600 r/min for 5 minutes, so as to perform an external addition treatment, thereby providing a

TABLE 3

| Raw material                                  | Alcohol                              | Production Example |                    |                       |                       |
|-----------------------------------------------|--------------------------------------|--------------------|--------------------|-----------------------|-----------------------|
|                                               |                                      | Resin              |                    | Production Example C2 |                       |
|                                               |                                      | Resin C-1          | Resin C-2          | Production Example C1 | Production Example C2 |
|                                               |                                      | part by mol *1     | charged amount (g) | part by mol *1        | charged amount (g)    |
| monomer of polyester                          | 1,10-Decanediol                      | 100                | 2436               | 100                   | 2828                  |
| component                                     | 1,12-Dodecanediol                    |                    |                    | 100                   | 2828                  |
| Acid component                                | Sebacic acid                         |                    |                    |                       |                       |
|                                               | Dodecanedioic acid                   | 100                | 3220               | 0.5                   | 28                    |
| Esterification catalyst                       | Tin(II) 2-ethylhexanoate (% by mass) | 0.5                | 28                 | 0.5                   | 28                    |
| Promoter                                      | Gallic acid monohydrate (% by mass)  | 0.03               | 1.7                | 0.03                  | 1.7                   |
| Polyester segment/acrylic resin segment ratio |                                      |                    | 1.000              |                       | 1.000                 |
| Properties of resin                           | Acid value (mgKOH/g)                 |                    | 21.3               |                       | 23.5                  |
|                                               | Number average molecular weight (Mn) | 3800               |                    | 4100                  |                       |
|                                               | Softening point (°C.)                | 80.5               |                    | 84.3                  |                       |
|                                               | Melting point (°C.)                  | 78.6               |                    | 81.5                  |                       |
|                                               | Crystallinity index                  | 1.02               |                    | 1.03                  |                       |

\*1 molar number per 100 moles of total amount of alcohol component

## [Production of Toner for Electrophotography]

## Examples and Comparative Examples

100 parts by mass of a binder resin obtained by mixing the resins shown in Table 4, the polyhydroxyamine compound, 5 parts by mass of a colorant "Regal 330R" (produced by Cabot Corporation, carbon black), 1 part by mass of a negative charge controlling agent "LR-147" (produced by Japan Carlit Co., Ltd.), and 2 parts by mass of a release agent "NP-105" (produced by Mitsui Chemicals, Inc., propylene wax, melting point: 140° C.) were stirred with a Henschel mixer, and then melt-kneaded with a co-rotation twin screw extruder having a total length of the kneading part of 1,560 mm, a screw diameter of 42 mm, and a barrel inner diameter

toner having a volume median particle diameter ( $D_{50}$ ) of 6.5  $\mu\text{m}$ . The resulting toner was evaluated and shown in Table 4.

## (Addition Method of Polyhydroxyamine Compound)

The addition methods shown in the table are as follows.

Addition method A: added in the form of powder

Addition method B: added in the form of aqueous solution: 100 g of the polyhydroxyamine compound was dissolved in 200 g of ion exchanged water to prepare an aqueous solution of the polyhydroxyamine compound of 50% by mass.

The polyhydroxyamine compounds shown in the table are as follows.

PHA-1: 2-amino-2-hydroxymethyl-1,3-propanediol

PHA-2: 2-amino-2-hydroxyethyl-1,3-propanediol

PHA-3: 2-amino-2-methyl-1,3-propanediol

TABLE 4

|           | Binder resin |              |      |              | Polyhydroxyamine compound |                 | Addition method | rise ( $\mu\text{C/g}$ ) | Odor suppression |
|-----------|--------------|--------------|------|--------------|---------------------------|-----------------|-----------------|--------------------------|------------------|
|           | Kind         | part by mass | Kind | part by mass | Kind                      | part by mass *1 |                 |                          |                  |
| Example 1 | H-1          | 70           | L-1  | 25           | C-1                       | 5               | PHA-1           | 0.5                      | A                |
| Example 2 | H-1          | 70           | L-1  | 25           | C-1                       | 5               | PHA-1           | 2                        | A                |
| Example 3 | H-1          | 70           | L-1  | 25           | C-1                       | 5               | PHA-1           | 0.05                     | A                |
| Example 4 | H-1          | 70           | L-1  | 25           | C-1                       | 5               | PHA-2           | 0.5                      | A                |
| Example 5 | H-1          | 70           | L-1  | 25           | C-1                       | 5               | PHA-3           | 0.5                      | A                |

TABLE 4-continued

|             | Binder resin |              |      | Polyhydroxyamine compound |      |              | Charge |                 |                 |             |                  |
|-------------|--------------|--------------|------|---------------------------|------|--------------|--------|-----------------|-----------------|-------------|------------------|
|             | Kind         | part by mass | Kind | part by mass              | Kind | part by mass | Kind   | part by mass *1 | Addition method | rise (μC/g) | Odor suppression |
| Example 6   | H-1          | 70           | L-1  | 25                        | C-1  | 5            | PHA-1  | 0.5             | B               | 0.97        | 3.7              |
| Example 7   | H-2          | 70           | L-1  | 25                        | C-1  | 5            | PHA-1  | 0.5             | A               | 0.89        | 3.6              |
| Example 8   | H-3          | 70           | L-1  | 25                        | C-1  | 5            | PHA-1  | 0.5             | A               | 0.86        | 3.3              |
| Example 9   | H-4          | 70           | L-1  | 25                        | C-1  | 5            | PHA-1  | 0.5             | A               | 0.82        | 3.1              |
| Example 10  | H-5          | 70           | L-3  | 25                        | C-1  | 5            | PHA-1  | 0.5             | A               | 0.8         | 2.8              |
| Example 11  | H-1          | 70           | L-2  | 25                        | C-1  | 5            | PHA-1  | 0.5             | A               | 0.95        | 3.7              |
| Example 12  | H-1          | 70           | L-1  | 25                        | C-2  | 5            | PHA-1  | 0.5             | A               | 0.93        | 3.8              |
| Example 13  | H-1          | 70           | L-1  | 30                        | —    | —            | PHA-1  | 0.5             | A               | 0.87        | 3.8              |
| Example 14  | H-6          | 70           | L-4  | 25                        | C-1  | 5            | PHA-1  | 0.5             | A               | 0.79        | 3.0              |
| Comparative | H-1          | 70           | L-1  | 25                        | C-1  | 5            | —      | —               | —               | 0.53        | 1.2              |
| Example 1   |              |              |      |                           |      |              |        |                 |                 |             |                  |
| Comparative | H-1          | 70           | L-1  | 25                        | C-1  | 5            | PHA-1  | 7               | A               | 0.64        | 3.8              |
| Example 2   |              |              |      |                           |      |              |        |                 |                 |             |                  |

\*1 blended amount (part by mass) per 100 parts by mass of binder resin

It can be understood from the above that the toners for electrophotography of Examples of the present invention exhibit an excellent charge rise property by containing the particular polyhydroxyamine compound, as compared to the toners for electrophotography of Comparative Examples.

The invention claimed is:

1. A toner for electrophotography, comprising a binder resin, and a polyhydroxyamine compound represented by the following formula (1) in an amount of 0.001 part by mass or more and 5.0 parts by mass or less per 100 parts by mass of the binder resin:



(1) 35

wherein R<sup>1</sup> represents a hydroxyalkyl group having a number of carbon atoms of 1 or more and 5 or less; R<sup>2</sup> represents a hydrogen atom, an alkyl group having a number of carbon atoms of 1 or more and 6 or less, or a hydroxyalkyl group having a number of carbon atoms of 1 or more and 5 or less; and R<sup>3</sup> and R<sup>4</sup> each represent an alkanediyl group having a number of carbon atoms of 1 or more and 5 or less, provided that R<sup>3</sup> and R<sup>4</sup> may be the same as or different from each other.

2. The toner for electrophotography according to claim 1, wherein the polyhydroxyamine compound is at least one selected from the group consisting of 2-amino-2-hydroxymethyl-1,3-propanediol and 2-amino-2-hydroxyethyl-1,3-propanediol.

3. The toner for electrophotography according to claim 1, wherein the polyhydroxyamine compound is 2-amino-2-hydroxymethyl-1,3-propanediol.

4. The toner for electrophotography according to claim 1, further comprising a charge controlling agent.

5. The toner for electrophotography according to claim 1, comprising one selected from the group consisting of a polyester and a composite resin having a polyester segment as the binder resin.

6. The toner for electrophotography according to claim 5, wherein an alcohol component of the polyester contains an alkylene oxide adduct of bisphenol A.

7. The toner for electrophotography according to claim 1, wherein the binder resin has a number average molecular weight of 1,000 or more and 7,000 or less.

25 8. The toner for electrophotography according to claim 1, wherein the binder resin has a softening point of 90° C. or more and 160° C. or less.

30 9. A process for producing a toner for electrophotography, comprising: melt-kneading a toner raw material mixture comprising a binder resin, and a polyhydroxyamine compound represented by the following formula (1) in an amount of 0.001 part by mass or more and 5.0 parts by mass or less per 100 parts by mass of the binder resin; and pulverizing a resulting melt-kneaded material:



(1)

40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335

14. The process for producing a toner for electrophotography according to claim 13, wherein an alcohol component of the polyester contains an alkylene oxide adduct of bis-phenol A.

15. The process for producing a toner for electrophotography according to claim 9, wherein the binder resin has a number average molecular weight of 1,000 or more and 7,000 or less. 5

16. The process for producing a toner for electrophotography according to claim 9, wherein the binder resin has a 10 softening point of 90° C. or more and 160° C. or less.

\* \* \* \* \*